

## UNITED STATES PATENT OFFICE

1,930,956

## ACID RESISTING ALLOY

Reginald Hazeltine, Chicopee Falls, Mass.

No Drawing. Application January 18, 1933  
Serial No. 652,421

2 Claims. (Cl. 75—1)

This invention relates to an alloy composed mainly of copper and silicon and containing sufficient chromium to give a high tensile strength and satisfactory machining properties.

5 The chief object of my invention is to provide an alloy that is extremely resistant to the chemical action of mineral and organic acids and other corrosive liquids which are present in varying degree in all natural water supplies and that at 10 the same time, possesses those physical properties which permit hot rolling, drawing and shaping combined with a high tensile strength, which will permit of its practical use in the manufacture of articles destined to be subjected to the action 15 of corrosive liquids.

I have discovered that by combining copper with silicon in certain proportions an alloy is obtained having high resistance to corrosive liquids and exceptionally fine rolling characteristics.

20 While the addition of silicon up to 3% is desirable I have found that when this percentage is increased to 5% the alloy is brittle and does not possess the desired rolling characteristics. I have found that the low percent silicon alloy 25 (3% or under) while possessing certain desired characteristics from the standpoint of the rolling mill, did not have the desired tensile strength and good machining qualities. It is possible however to obtain all the desired characteristics 30 by the addition of from  $\frac{1}{8}$  to  $\frac{1}{4}$  of one percent chromium to this silicon copper alloy.

The alloy made in accordance with my invention may be described as having a base of copper to which appreciable amounts of chromium and 35 silicon have been added for the specific purposes above noted, the silicon predominating the chromium. The alloy contains no other elements except a small amount of iron and incidental impurities, introduced with the chromium and silicon.

40 Alloys containing from 2 to 3% of silicon with

from  $\frac{1}{8}$  to  $\frac{1}{4}$  of one percent chromium are characterized physically by a high tensile strength, 45,000 to 48,000 lbs. per sq. inch ultimate strength in a cast bar, and 55,000 to 60,000 lbs. per sq. inch in a rolled strip, and possesses an elongation before fracture of from 53 to 58%. Also characteristics that permit the metal to be rolled into thin sheets or pressed and drawn into shapes of considerable depth.

These alloys may be produced by melting a given weight of copper and adding to it pure refined silicon and an alloy of chromium copper or it may be made by alloying chromium and copper at a high temperature and adding pure refined silicon. It is advisable to protect the melting metal from oxidation by the addition of a small amount of charcoal as is done in ordinary foundry practice.

The above combination of copper, silicon and 75 chromium may be regarded as a type of bronze and be designated as a silicon chromium bronze, and be handled in the foundry as any ordinary phosphor bronze of 90 parts copper and 10 parts phosphor-tin. The ordinary deoxidizers such as 80 phosphor copper or boron copper may be used as on the more common bronzes.

This alloy is characterized chemically by the extreme resistance to acids and corroding liquids that are the characteristics of the elements that make it up and is especially useful as a material 85 for tanks, range boilers, pipes and other apparatus often subjected to the corrosive action of impure water.

I claim:

1. A copper base alloy containing 3% silicon,  $\frac{1}{4}$  of one percent chromium and the balance 90 commercially pure copper.

2. A copper base alloy containing  $1\frac{1}{2}$  to 5% silicon and  $\frac{1}{8}$  to 1% chromium the balance being 95 commercially pure copper.

REGINALD HAZELTINE.